

Jan. 27, 1942.

E. LIONNE

2,271,458

RUBBER IMPREGNATED AND COATED WEB

Filed Jan. 3, 1936



## UNITED STATES PATENT OFFICE

2,271,458

## RUBBER IMPREGNATED AND COATED WEB

Ernest Lionne, Lynn, Mass.

Application January 3, 1936, Serial No. 57,395

10 Claims. (Cl. 91—68)

This invention relates to the combined impregnation and coating of porous materials such as textile fabrics with rubber in the initial form of rubber latex in one operation.

Heretofore in the coating of sheet materials, such as textile fabrics, with rubber solutions, that is, a solution of rubber in a suitable solvent therefor, the tensioned moving web of sheet material has been passed under a coating or spreading knife or bar in front of which is a pool of the coating material which is spread onto the surface of the material by the knife. In this manner a layer of the coating material is deposited on the surface of the web. If the web is a closely woven fabric it can be coated but the coating material because of its relatively high viscosity does not pass into the web but exists only on the surface of the web. If the web is sufficiently loosely woven it can be impregnated, that is to say, the coating material occupies mainly the interstices of the weave but there is relatively no coating of the material on the surface. If the web has an open weave the coating material merely passes through the web without either impregnating or coating it. Some weaves, such as those that are not too loosely woven can be impregnated and coated in two successive operations wherein the web is first impregnated, and then dried to evaporate the volatile solvent from the impregnating solution and then coated in the manner above described. Furthermore, webs that are loosely woven, as, for instance, textile fabrics of the nature of cheese or tobacco cloth, cannot be impregnated and coated because the interstices of the weave are so great that they cannot be filled and at the same time receive and support a surface coating by any commercially practicable single operation known heretofore.

Hence an object of the present invention is a process, and a machine for carrying out the process, wherein webs of sheet material, and particularly textile fabrics, can be impregnated and coated in one operation by a rubber film forming material.

In many instances it is not essential that the coated fabric should be at the same time completely impregnated and for many purposes it is desirable to have the strands of the fabric covered with a thin film of rubber for bonding the fabric to the coating layer while leaving the interstices of the weave, that is to say, the spaces between the strands of the fabric, open except at the coated face, where they are traversed by the coating. This is desirable, for instance, in

the waterproofing of fabrics for raincoats and the like, and the manner in which this result is secured constitutes a further object of the invention.

In the manufacture of raincoats, for instance, and especially raincoats for women, it is desirable to employ fabrics having pleasing surface designs and weaves. Heretofore, however, when such fabrics have been treated to render them waterproof, such designs and weaves have deleteriously obscured by the overlying waterproofing material. Hence a further object of the invention is the provision of a waterproof fabric the outer or weather surface of which is not harmfully covered or obscured by the waterproofing material and wherein the outer surface presents substantially no evidence of the waterproof nature of the material.

In the performance of my process for making my impregnated and coated fabric I use rubber latex as the rubber-film forming impregnating and coating material. By the term rubber latex I mean the usual dispersion of rubber-like particles of any of the varieties of rubber, including gutta-percha, balata and the like, in their natural liquid form, although the latex may be concentrated and may contain a stabilizer to maintain the rubber-like particles in dispersed condition, and for some purposes a vulcanizing agent or agents. For many purposes and particularly for waterproofing garments the rubber latex is as transparent as is practicable, although for other purposes the rubber latex may contain a filler or a pigment. Rubber latex is characterized by a high rubber content and low viscosity. Unconcentrated rubber latex can be obtained having as high as 60% or more of rubber with a viscosity of not more than four times that of water. A rubber solution, on the other hand, made by dissolving rubber in a suitable solvent has great viscosity and a much lower rubber content. For some purposes the viscosity of the rubber latex is undesirably low and I increase its viscosity by adding thereto a viscosity increasing medium as a mucilage. Karaya gum, casein, for instance, are suitable mediums.

In the performance of my process, instead of passing a tensioned web under a coating knife I support the practically untensioned web on a carrier belt characterized by having a fabric receiving surface that is not strongly adherent to the rubber film so that the dry coated fabric readily can be detached therefrom. The surface of the carrier belt preferably is as smooth and bright as is practicable so as to impart to the

surface coating of the web a smooth appearance. Preferably the belt is composed of artificial leather having a smooth bright surface coating thereon, which supports the fabric during the process of impregnation and coating. This manner of supporting and treating the fabric constitutes another object of the invention.

The coating and impregnating material is so applied that rubber latex is present mainly in the lower part of the web and between the belt and the fabric so that when the liquid content of the latex is removed a solid continuous sheet of rubber is formed on the lower surface of the web and between it and the belt. Such manner of treating the fabric constitutes a further object of the invention.

Another object of the invention is a fabric having on one face thereof a substantially continuous layer of coated material, the material of the layer also existing as thin films around the strands of the fabric but the other surface of the fabric preferably being free from any continuous coating.

A further object of the invention is the combined and simultaneous impregnation and coating of a fabric by supporting the fabric on a suitable support and applying to the fabric a quantity of the latex that is greater than that which the fibre of the fabric can absorb so that the excess latex will collect in the interstices of the lower part of the fabric and between it and the web and form the coating for the fabric.

A further object of the invention is generally to improve upon coating processes.

Fig. 1 is a diagrammatic view of a coating and impregnating machine constructed for the performance of the process of my invention.

Fig. 2 is a sectional view illustrating in enlarged form the application of the film forming material to the fabric.

Fig. 3 is a view similar to Fig. 2 but illustrating a modification where the film forming material is introduced between the fabric and the supporting belt.

Fig. 4 is a plan view of a portion of a coated fabric embodying the present invention.

Fig. 5 is an enlarged sectional view of the fabric taken along line 5—5 of Fig. 4.

Fig. 6 is an enlarged sectional view of the latex containing fabric on the supporting belt.

The coating and impregnating machine forming a part of the present invention, as illustrated in Fig. 1, includes an endless web supporting belt 10 passing about end supporting rolls 12 and 14, one or both of which may be driving rolls, and having an upper horizontal pass adjacent the driving roll 12 and passing over suitably positioned guide and supporting rolls 16 into and out of a drying chamber 28, which can be heated by suitable means, not illustrated, to evaporate the volatile constituents of the rubber latex.

The fabric 22 to be coated is contained in a roll 24 and passes from said roll over a supporting roll 26 and preferably first into a conditioning tank 28 where it passes under the surface of a liquid bath 30 in said tank and between a plurality of sets of squeeze rolls 32 which drive the conditioning liquid into and thus thoroughly impregnates the fabric with the liquid. The conditioning liquid may consist simply of water either alone or containing some reagent which governs the ability of the fabric to take up the rubber latex. The fabric passes out of the trough and between a set of wringer rolls 34

which express surplus liquid therefrom. The fabric thence passes over a guide roll 36 which is elevated suitably above the top horizontal pass of the conveyor belt 10 and thence onto the surface of the conveyor belt under the coating knife 38. The conveyor belt on opposite sides of the coating knife or bar 38 is supported on rolls 40 and the knife is set below the tops of said rolls so that the conveyor belt and the fabric thereon is depressed into a trough-like formation, as is shown in the enlarged view in Fig. 2. The depth of the trough and hence the degree of pressure exerted on the fabric by the knife can be regulated by adjusting the vertical height of the knife in a well known manner. The angle of the knife with respect to the fabric can be adjusted also.

A body or pool 42 of rubber latex is maintained in front of the coating knife and upon the fabric and the belt, latex being constantly added to the body 42 through a pipe 44 from a suitable tank 46, the flow being controlled by suitable means as a valve 48. The coating knife spreads the rubber latex over the surface of the fabric and into and through the fabric and onto the belt in a manner which will be described in greater detail hereinafter. The coated and impregnated fabric thence is carried forward by the supporting belt 10. For some purposes it may be desirable to provide another coating knife 50 for further spreading on the surface of the fabric and forcing into the fabric the material laid thereon by the first knife.

The wet coated material thence passes with the conveyor belt into the heated drying chamber 28 where the volatile constituents of the rubber latex are evaporated. At the exit of the drying chamber the lower pass of the conveyor belt passes over a guide roll 48. At this point the coated fabric is detached or stripped from the belt and is passed around a guide roll 52 and thence over one or more heated drums 54, two being here shown, that are heated sufficiently high to vulcanize the rubber film. The fabric thence passes from the last vulcanizing drum and is wound into a roll 56. Instead of using an unvulcanized latex, which, for vulcanizing, necessitates the vulcanizing drums, or equivalent, a vulcanized latex can be used with satisfactory results and the drums can be eliminated.

The action of the coating knife is illustrated more particularly in Figs. 2 and 6. Referring particularly to Fig. 6, the damp fabric 22 having the warp strands A and the weft strands B is supported on the upper pass of the conveyor belt 10 on the smooth coated face 38 thereof and passes under the knife 38 where the belt dips between the supporting rollers 40 to form a trough for the pool 42 of latex. The fabric passes beneath the latex pool and the latex due to its high fluidity passes through the fabric so that at the point where the fabric is directly under the knife the fabric is substantially completely filled with rubber latex, as indicated by the shaded section 60. The fabric passes upwardly with the belt out of the trough to the front supporting roll 40 where the belt passes on horizontally. The latex remains on the fabric during this upward pass without any appreciable tendency to flow downwardly toward the knife because of the resistance to its flow offered by the web of the fabric and also due to the speed of the belt. The fabric, under the knife, is compressed to an extent determined by the pressure between the fabric and knife so that the fabric is thinner under the knife

than its normal uncompressed thickness. Thus the fabric expands after leaving the knife and the rubber latex does not completely fill the interstices of the uncompressed fabric. On the horizontal pass of the belt the latex settles to the lower part of the fabric, partly by gravity and partly by capillary action between the belt and fabric or assumes some such position as illustrated at the right hand part of Fig. 6. The latex also collects under the fabric and between the warp strands and the belt by capillary action so that the fabric is upon a thin film 62 of rubber latex.

The amount of latex in the interstices of the fabric can be adjusted by adjusting the pressure between the fabric and knife, which adjusts the degree of compression of the fabric and hence the amount of latex that the compressed fabric can accommodate. The amount of rubber in the fabric can be widely adjusted by the use of latices of different concentrations.

The belt with the fabric and latex then passes into the evaporating or drying chamber 20 where the moisture content of the rubber latex is dissipated and the rubber film is formed.

A section of the coated fabric is illustrated in Fig. 5 wherein the fabric 22 has the rubber coating 64 on its bottom face formed by the coagulation of the rubber in the latex film 62. The thickness of the rubber coating is, of course, less than the thickness of the rubber latex under the fabric and on the horizontal pass of the belt due to the evaporation of the liquid content of the latex. The rubber coating 64 may have a thickness approximately equal to 40 to 50% of the thickness of the latex layer under the fabric depending upon the proportion of solid matter to liquid in the latex. Thin films 66 of rubber cover the fabric strands in the top face of the fabric and these films are integral with the coating 64. The films, however, are so thin that there is no rubber coating readily apparent from a casual inspection of the top surface. Thus the weave of the fabric and the pattern or design thereon is substantially unobscured.

In the modification illustrated in Fig. 3 the rubber latex 42a is deposited directly upon the belt under the fabric in front of the knife. The action of the knife is thus to force the rubber latex positively through the fabric so as to insure thorough penetration of the fabric by the latex. The latex also collects between the fabric and the knife so that the fabric passes through the pool of latex. This arrangement is sometimes desirable for impregnating and coating especially closely woven or thick fabrics.

For the coating and impregnating of certain webs where the viscosity of the rubber latex is too little to obtain the intended results I may desire to increase the viscosity by adding to the latex a suitable medium as a mucilage in amounts sufficient to obtain the desired increase in viscosity.

In passing through the latex pool in front of the coating knife, the strands of the fabric and the fibres of the strands absorb the latex, the strands at least becoming substantially saturated. The interstices of the fabric also receive latex and the latex in the interstices collects in the lower part of the fabric and between it and the supporting belt. It is important that the fabric be treated with more than enough latex than the strands and fibres can absorb; and the excess in part forms the surface coating. No coating will be

formed if all the latex applied to the fabric can be absorbed by the strands and fibres.

As an example of what is considered good practice in the performance of the invention for making waterproof fabric for women's raincoats, percale weighing 100 grams per square yard and having a count of 80 x 80 and a thickness of eight thousandths of an inch, is treated to have deposited thereon and therein 3 to 3½ ounces (85 to 100 grams) of rubber per square yard. The material is entirely waterproof and there is no material evidence of rubber on the outer surface or face thereof. If the rubber deposit is increased to 4 ounces (114 grams) shiny surfaces of rubber film begin to appear on the surface, which surface films are not desired. A plaid, weighing 47 grams per square yard, and having a count of 76 x 76, and a thickness of seven and one-half thousandths of an inch, is satisfactorily waterproofed by a rubber deposit of from 2 to 2½ ounces (57 to 71 grams) and surface films of rubber appear on the face with a rubber deposit of around 3 ounces.

It is the cloth itself and not the adjustment of the machine that determines to a considerable extent the amount of rubber deposited in and on the cloth. If the fabric is of such nature that, to obtain a desirable coating, the outer face of the fabric has shiny spots indicative of surface films, then the latex which forms these spots has to be removed as by the use of a second knife 50. The amount of rubber latex absorbed by the fabric depends upon many factors such as the weight and character of the fabric and the prior chemical treatment, including printing, that the fabric has received. In general, however, the weight of the fabric is the major factor determining the amount of rubber latex, and consequently rubber absorbed by the fabric and the heavier the fabric the more latex it absorbs. In the examples above given the rubber deposit in and on the plaid is greater in proportion to the weight of the fabric than with the percale. The plaid, however, has a somewhat lower count and a more open weave than the percale so that the additional rubber is represented by that part that is in the coating and in the interstices of the weave.

I claim:

1. The method of coating and impregnating a pervious fabric which comprises conveying the fabric on a horizontal travelling supporting surface, applying a coating and impregnating liquid to the fabric in a quantity greater than the fabric can absorb so that excess liquid collects as a liquid sheet on the supporting surface under and in contact with the fabric and travels with the surface and fabric, and drying the liquid sheet to form a solid sheet adherent to the fabric while the underlying liquid is retained against the fabric by the supporting surface.
2. The method as in claim 1 wherein the coating and impregnating liquid comprises rubber latex.
3. The method of impregnating and coating a pervious fabric which comprises passing an impregnating and coating liquid in a quantity greater than the fabric can absorb through the fabric on a yieldable supporting surface to collect excess liquid as a liquid sheet on the surface under the fabric by moving the fabric having an impregnating and coating liquid on its upper surface under a spreader knife which exerts pressure thereon, moving the yieldable supporting surface with the fabric to facilitate unitary move-

ment of the liquid sheet and fabric, and drying the liquid in and under the fabric to form a solid sheet on and adherent to the under face of the fabric.

4. The method of rubber coating and impregnating simultaneously an absorbent pervious fibrous fabric on a smooth impervious supporting surface, which method comprises applying to the upper surface of the fabric rubber latex in a quantity greater than that which the fibres of the fabric can absorb, forcing the excess latex into and through the fabric to occupy the interstices of the fabric and collect in the lower part thereof and form a liquid sheet between the fabric and the supporting surface, eliminating the liquid content of the latex to convert the latex in the fabric to solid rubber and the latex in the liquid sheet to a solid sheet which is on the lower face of the fabric and is integral with the rubber in the body of the fabric, and detaching the impregnated and coated fabric from the supporting surface.

5. That method of producing a rubber coated fabric comprising the steps of simultaneously applying both an open woven fabric and liquid latex to a yieldable horizontal moving surface to which a dried film of latex will not adhere, forcing sufficient latex into and through the fabric to form a pool under the fabric, passing the plied fabric latex and surface through a drying medium to produce a rubber film on the surface, which film is attached to the fabric, and finally removing the fabric from the surface with the dried rubber coating adhered to the lower side of the fabric.

6. That method of producing a rubber coated fabric comprising the steps of applying a pervious fabric to an impervious supporting surface to which a dried film of latex rubber will not adhere, drawing the fabric and its associated supporting surface under a spreader knife having latex associated with the leading edge thereof to force latex into and through the fabric, the knife forcing sufficient latex through the fabric to form a pool of latex between same and the supporting surface, moving the pool of latex, fabric, and supporting surface as a unit and drying the plied fabric and latex to form a rubber sheet on the under surface of the fabric, and removing the fabric and its associated sheet from its supporting surface.

7. That method of producing a rubber coated fabric comprising the steps of applying an open mesh fabric to a yieldable moving impervious supporting surface, associating a volume of latex with the upper surface of the fabric, moving the

plied fabric and supporting surface underneath spreader means to force the latex into and through the fabric and form a pool underneath the fabric, passing the plied fabric latex and supporting surface through a drying medium to form a rubber coating on the lower surface of the fabric, and removing the fabric and its rubber coat from the supporting surface.

8. The method of simultaneously rubber coating and impregnating an absorbent pervious fibrous fabric on a yieldable smooth impervious supporting surface, which method comprises applying to the upper surface of the fabric rubber latex in a quantity greater than that which the fibres of the fabric can absorb, forcing the excess latex into and through the fabric to occupy the interstices thereof and collect in the lower part of the fabric and form a liquid sheet between the fabric and the supporting surface, 15 passing the plied supporting surface latex pool and fabric as a unit through a drying medium to convert the latex in the fabric to solid rubber and the latex in the liquid sheet to a solid sheet which is on the lower face of the fabric and is integral with the rubber in the body of the fabric, and detaching the impregnated and coated fabric from the supporting surface.

9. The method of coating a pervious fabric with rubber, which method comprises associating the fabric with a horizontal traveling surface to which a dried film of latex will not adhere, forming a pool of latex in a quantity greater than the fabric can absorb between the fabric and the supporting surface, moving the pool of latex and fabric as a unit with the horizontal traveling surface, passing the plied latex pool, fabric and supporting surface as a unit through a drying medium to dry the latex and form a solid rubber sheet adhered to the fabric, and removing the fabric and rubber sheet as a unit from the moving surface.

10. The method of coating a pervious fabric with rubber, which method comprises associating the fabric with a yieldable horizontal traveling surface to which a dried film of latex will not adhere, drawing the fabric and surface under a spreader, forcing latex in a quantity greater than the fabric can absorb into and through the fabric to form a pool between the fabric and the supporting surface, moving the pool of latex and fabric as a unit with the horizontal traveling surface, and passing the plied latex pool, fabric and supporting surface through a drying medium to dry the latex and form a solid rubber sheet adhered to the fabric.

ERNEST LIONNE.